



US005244594A

# United States Patent [19]

Favre et al.

[11] Patent Number: 5,244,594  
[45] Date of Patent: \* Sep. 14, 1993

[54] BLEACH ACTIVATION MULTINUCLEAR MANGANESE-BASED COORDINATION COMPLEXES

[75] Inventors: Thomas L. F. Favre, Pijnacker; Ronald Hage, Leiden; Karin Van der Helm-Rademaker, Vlaardingen; Jean H. Koek, Vlaardingen; Rudolf J. Martens, Vlaardingen; Ton Swarthoff, Hellevoetsluis; Marten R. P. van Vliet, Haarlem, all of Netherlands

[73] Assignee: Lever Brothers Company, Division of Conopco, Inc., New York, N.Y.

[\*] Notice: The portion of the term of this patent subsequent to Sep. 21, 2010 has been disclaimed.

[21] Appl. No.: 703,555

[22] Filed: May 21, 1991

## [30] Foreign Application Priority Data

May 21, 1990 [GB] United Kingdom ..... 9011338  
Dec. 18, 1990 [GB] United Kingdom ..... 9027415

[51] Int. Cl.<sup>5</sup> ..... C01B 15/00; C09K 3/00

[52] U.S. Cl. ..... 252/186.33; 252/186.42; 252/186.43; 252/186.25; 252/186.21; 252/95; 252/174.12

[58] Field of Search ..... 252/186.21, 186.22, 252/186.33, 186.42, 186.43

## [56] References Cited

### U.S. PATENT DOCUMENTS

4,728,455 3/1988 Rerek ..... 252/99  
5,021,187 6/1991 Harriott et al. ..... 252/186.38 X  
5,114,606 5/1992 van Vliet et al. ..... 252/103 X  
5,114,611 5/1992 van Kralingen et al. ... 252/186.33 X

## FOREIGN PATENT DOCUMENTS

0369841 5/1990 European Pat. Off.

## OTHER PUBLICATIONS

J. Am. Chem. Soc. (Wieghardt et al.), 1988, vol. 110, pp. 7398-7411.

J. Chem. Soc., Chem. Soc., (Wieghardt et al.), 1988, pp. 1145-1146.

CA 112(19): 177773r, Beck Warren F. et al. Dept. Chem., Yale University, USA.

CA 105(26): 237364w, Wieghardt, Karl; Ruhr-University, Bochum D-4630 Fed. Rep. Germany.

Primary Examiner—Richard D. Lovering

Assistant Examiner—Joseph D. Anthony

Attorney, Agent, or Firm—Milton L. Honig

## [57] ABSTRACT

Novel bleach and oxidation catalysts, a method of bleaching substrates using these catalysts and bleaching (detergent) compositions containing the catalysts are reported.

The catalysts are a manganese-based co-ordination complex of the general formula:



wherein Mn is manganese in the IV-oxidation state; n and m are independent integers from 2-8; X represents a co-ordination or bridging species; p is an integer from 0-32; Y is a counter-ion, the type of which is dependent on the charge z of the complex which can be positive, zero or negative; q=z/[charge Y]; and L is a ligand which is an organic molecule containing a number of hetero-atoms selected from N, P, O, and S, which coordinates via all or some of its hetero-atoms and/or carbon atoms to the Mn<sup>IV</sup>-center(s), which latter are anti-ferromagnetically coupled.

19 Claims, No Drawings

BLEACH ACTIVATION MULTINUCLEAR  
MANGANESE-BASED COORDINATION  
COMPLEXES

This relates to activation of bleaches employing peroxy compounds, including hydrogen peroxide or a hydrogen peroxide adduct, which liberate hydrogen peroxide in aqueous solution, as well as peroxy acids; to compounds that activate or catalyst peroxy compounds; to bleach compositions including detergent bleach compositions which contain a catalyst for peroxy compounds; and to processes for bleaching and/or washing of substrates employing the aforementioned types of compositions.

In particular, the present invention is concerned with the novel use of manganese compounds as improved catalyst for the bleach activation of peroxy compound bleaches.

Peroxide bleaching agents for use in laundering have been known for many years. Such agents are effective in removing stains, such as tea, fruit and wine stains, from clothing at or near boiling temperatures. The efficacy of peroxide bleaching agents drops off sharply at temperatures below 60° C.

It is known that many transition metal ions catalyst the decomposition of  $H_2O_2$  and  $H_2O_2$ -liberating per-compounds, such as sodium perborate. It has also been suggested that transition metal salts together with a chelating agent can be used to activate peroxide compounds so as to make them usable for satisfactory bleaching at lower temperatures.

For a transition metal to be useful as a bleach catalyst in a detergent bleach composition, the transition metal compound must not unduly promote peroxide decomposition by non-bleaching pathways and must be hydrolytically and oxidatively stable.

Hitherto the most effective peroxide bleach catalysts are based on cobalt as the transition metal.

The addition of catalysts based on the transition metal cobalt to detergent formulations is, however, a less acceptable route as judged from an environmental point of view.

In a number of patents the use of the environmentally acceptable transition metal manganese is described. All 45 these applications are, however, based on the catalysing action of the free manganese ion and do not fulfil the requirement of hydrolytic stability. U.S. Pat. No. 4,728,455 discusses the use of Mn(III)-gluconate as peroxide bleach catalyst with high hydrolytic and oxidative stability; relatively high ratios of ligand (gluconate) to Mn are, however, needed to obtain the desired catalytic system. Moreover, the performance of these Mn-based catalysts is inadequate when used for bleaching in the low-temperature region of about 20°-40° C., and 55 they are restricted in their efficacy to remove a wide class of stains.

We have now discovered a certain class of manganese-based co-ordination complexes which fulfil the demands of stability (both during the washing process and in the dispenser of the washing machine), and which are extremely active, even in the low-temperature region, for catalyzing the bleaching action of peroxy compounds on a wide variety of stains.

It is therefore an object of the present invention to 65 provide a manganese-based co-ordination complex, or a precursor therefor as an improved catalyst for the bleach activation of peroxy compounds, including hy-

drogen peroxide and hydrogen peroxide-liberating or -generating compounds, as well as peroxyacid compounds including peroxyacid precursors, over a wide class of stains at lower temperatures.

5 Another object of the invention is to provide an improved bleaching composition which is effective at low to medium temperatures of e.g. 10°-40° C.

Still another object of the invention is to provide new, improved detergent bleach formulations, which are especially effective for washing at lower temperatures.

Yet another object of the invention is to provide aqueous laundry wash media containing new, improved detergent bleach formulations.

15 A further object of the invention is to provide an improved bleaching system comprising a peroxy compound bleach and a manganese-based co-ordination complex (or a precursor therefor) for the effective use in the washing and bleaching of substrates, including laundry and hard surfaces (such as in mechanical dishwashing, general cleaning etc.) and in the textile, paper and woodpulp industries and other related industries.

The present catalysts of the invention may also be applied in the peroxide oxidation of a broad range of organic molecules such as olefins, alcohols, aromatic ethers, sulphoxides and various dyes, and also for inhibiting dye transfer in the laundering of fabrics.

These and other objects of the invention, as well as further understandings of the features and advantages thereof, can be had from the following description.

The active catalyst according to the invention is a well-defined manganese(IV)-based co-ordination complex, consisting of a number of manganese atoms and a number of ligands, wherein the manganese centers are in the oxidation state IV and the Mn(IV)-centers are coupled anti-ferromagnetically. The extent of anti-ferromagnetic coupling is usually expressed as the exchange coupling parameter J. This parameter is negative for an anti-ferromagnetic interaction. (Anti-ferromagnetic coupling of transition metal ions is described, e.g., by R. S. Drago in "Physical Methods in Chemistry", 1977, Chapter 11, page 427 et seq. and for manganese in oxidation state (IV) by K. Wieghardt et al in "The Journal of the American Chemical Society", 1988, Vol. 110, pages 7398-7411).

The active manganese complex catalyst is of the following general formula (A):



in which

Mn is manganese in the IV-oxidation state and wherein n and m are independent integers from 2-8;

X represents a co-ordinating or bridging species such as  $H_2O$ ,  $OH^-$ ,  $O_2^{2-}$ ,  $O^{2-}$ ,  $HO_2^-$ ,  $SH^-$ ,  $S^{2-}$ ,  $>SO$ ,  $NR_2^-$ ,  $RCOO^-$ ,  $NR_3$ , with R being H, alkyl, aryl (optionally substituted),  $Cl^-$ ,  $N_3^-$ ,  $SCN^-$ ,  $N^3^-$  etc. or a combination thereof;

p is an integer from 0-32, preferably from 3-6; Y is a counter-ion, the type of which is dependent on the charge z of the complex; z denotes the charge of the charge z of the complex; z denotes the charge of the complex and is an integer which can be positive or negative. If z is positive, Y is an anion such as  $Cl^-$ ,  $Br^-$ ,  $I^-$ ,  $NO_3^-$ ,  $ClO_4^-$ ,  $NCS^-$ ,  $PF_6^-$ ,  $RSO_3^-$ ,  $RSO_4^-$ ,  $CF_3SO_3^-$ ,  $BPh_4^-$ ,  $OAc^-$  etc; if z is negative, Y is a common cation such as an

alkali metal, alkaline earth metal or (alkyl)ammonium cation etc.;  $q=z/[\text{charge Y}]$ ; L is a ligand which is an organic molecule containing a number of hetero-atoms (e.g. N, P, O and S, etc.), which co-ordinates via all or some of its hetero-atoms and/or carbon atoms to the Mn(IV)- center or centers, which are anti-ferromagnetically coupled. The extent of anti-ferromagnetic coupling  $|J|$  is preferably greater than  $200 \text{ cm}^{-1}$ , most preferably greater than  $400 \text{ cm}^{-1}$ .

As explained hereinbefore, the invention relates to the above-defined active manganese(IV)-based co-ordination complex including the precursors therefor.

A precursor for the class of active catalysts described can be any manganese co-ordination complex which, in the presence of a peroxy compound, is transformed into the active manganese complex of general formula A as defined above. The precursor molecule does not necessarily contain manganese in the oxidation state IV and the manganese centers are not necessarily anti-ferromagnetically coupled.

A preferred class of catalysts are the manganese complexes in which  $m=2$ ,  $n=2$ , and  $p=3$ , in which the manganese(IV)-centers are anti-ferromagnetically coupled. These are dinuclear manganese(IV)-complex compounds having the following general formula (B):



in which each X individually represents any of the bridging species described as co-ordinating ions in formula A above; and L, Y, q, and z are as described above. Suitable bridging species or co-ordinating ions normally have a donor atom and preferably are small-size molecules.

A more preferred class of catalysts are dinuclear manganese(IV)-complexes in which  $X=O^{2-}$  of formula (C):



wherein L, Y, q, and z are as described above.

#### The ligand L

L is an organic molecule with a number of hetero-atoms (like N, P, O, and S, etc.) which co-ordinates via all or some of its hetero-atoms and/or carbon atoms to the Mn(IV)-center.

A preferred class of ligands L are the multi-dentate ligands which co-ordinate via three hetero-atoms to the manganese(IV)-centers which are anti-ferromagnetically coupled, preferably those which co-ordinate via three nitrogen atoms to each one of the manganese(IV)-centers. The nitrogen atoms can be part of tertiary, secondary, or primary amine groups, but also part of aromatic ring systems, e.g. pyridines, pyrazoles, etc., or combinations thereof.

Not all ligands which co-ordinate via three N-atoms to one of the Mn(IV)-centers, however, will give rise to  $[LMn^{IV}(\mu-O)_3Mn^{IV}L]^z Y_q$  complexes; some give rise to complexes containing more or less than two manganese(IV)-centers. Only those ligands which have specific space-filling properties will give rise to the class of effective dinuclear Mn(IV)-complexes. This implies that by the definition of the more preferred catalyst  $[LMn^{IV}(\mu-O)_3Mn^{IV}L]^z$  also the space-filling properties

of the ligands L are important. Space-filling properties of the ligands can be derived by well-known techniques like molecular modelling and/or molecular graphics.

For example, less suitable ligands will give rise to  $L_2Mn$  mononuclear compounds (because of their insufficient space-filling properties, i.e. these ligands are too small) or will give rise to  $LMnX_3$  mononuclear compounds (because of their overly sufficient space-filling properties—these ligands are too big). Other less suitable ligands, though being tri-N-dentate ligands, will give rise to tetranuclear  $L_4Mn_4O_6$  clusters (because of their not entirely sufficient space-filling properties - a little too small).

Accordingly, those ligands having effective space-filling properties to give rise to  $LMn^{IV}(\mu-O)_3Mn^{IV}L$  clusters are most preferred.

Therefore, the most preferred class of catalysts are dinuclear manganese(IV)-complexes of formula (C), in which the manganese IV-centers are anti-ferromagnetically coupled, and wherein L contains at least three nitrogen atoms, three of which co-ordinate to each Mn(IV)-center. Representative for this class of catalysts are complexes of the formula (D):



in which  $L'N_3$  (and  $N_3L'$ ) represent ligands containing at least three nitrogen atoms.

Though Y can be any counter-ion as defined hereinbefore, the more preferred counter-ions Y are those which give rise to the formation of stable (with respect to hygroscopicity) solids. This means that their lattice-filling properties are compatible with the lattice-filling properties of the manganese cluster. Combinations of the more preferred manganese cluster with the counter-ion Y usually involve bigger counter-ions, such as  $ClO_4^-$ ,  $PF_6^-$ ,  $RSO_3^-$ ,  $RSO_4^-$ ,  $BPh_4^-$ ,  $OOCR^-$  (R=alkyl, aryl, etc., optionally substituted) etc.

Examples of suitable ligands L in their simplest forms are:

- (i) 1,4,7-trimethyl-1,4,7-triazacyclononane;
  - 1,4,7-trimethyl-1,4,7-triazacyclodecane;
  - 1,4,8-trimethyl-1,4,8-triazacycloundecane;
  - 1,5,9-trimethyl-1,5,9-triazacyclododecane.
  - (ii) Tris(pyridin-2-yl)methane;
  - Tris(pyrazol-1-yl)methane;
  - Tris(imidazol-2-yl)methane;
  - Tris(triazol-1-yl)methane;
  - (iii) Tris(pyridin-2-yl)borate;
  - Tris(triazol-1-yl)borate;
  - Tris(pyrazol-1-yl)borate;
  - Tris(imidazol-2-yl)phosphine;
  - Tris(imidazol-2-yl)borate.
  - (iv) 1,3,5-tris(aminomethyl)cyclohexane;
  - 1,1,1-tris(methylamino)ethane.
  - (v) Bis(pyridin-2-yl-methyl)amine;
  - Bis(pyrazol-1-yl-methyl)amine;
  - Bis(triazol-1-yl-methyl)amine;
  - Bis(imidazol-2-yl-methyl)amine,
- all optionally substituted on amine N-atom and/or  $CH_2$  carbon atom and/or aromatic ring.

Examples of preferred ligands are:

5  
-continuedwherein R is a C<sub>1</sub>-C<sub>4</sub> alkyl group.6  
-continued

wherein R can each be H, alkyl, or aryl, optionally substituted.

25 Examples of the most preferred catalysts are:

abbreviated as [Mn<sup>IV</sup><sub>2</sub>(μ-O)<sub>3</sub>(Me-TACN)<sub>2</sub>](PF<sub>6</sub>)<sub>2</sub>.abbreviated as [Mn<sup>IV</sup><sub>2</sub>(μ-O)<sub>3</sub>(me/Me-TACN)<sub>2</sub>](PF<sub>6</sub>)<sub>2</sub>.55 The anti-ferromagnetic coupling J value for these catalysts is ~ -780 cm<sup>-1</sup>.

Examples of precursors for the active catalysts are:



-continued

and



Both precursors, in the presence of a peroxy compound, will transform and give rise to the formation of the following active catalyst cation (1):



Any of these complexes, either preformed or formed in situ during the washing or bleaching process, are useful catalysts for the bleach activation of peroxy compounds over a wide class of stains at lower temperatures in a surprisingly much more effective way than any manganese- and cobalt-based catalysts hitherto known in the art. Furthermore, these catalysts exhibit a high stability against hydrolysis and oxidation. It should be noted that the catalytic activity is determined only by the  $[L_nMn_mX_p]^{z-}$  core complex and the presence of  $Y_q$  has hardly any effect on the catalytic activity.

Some of the complexes described in this invention have been prepared previously as scientific and laboratory curiosities, e.g. as models for naturally occurring Mn-protein complexes without bearing any practical function in mind (K. Wieghardt et al., Journal of American Chemical Society, 1988, 110 page 7398 and references cited therein, and K. Wieghardt et al., Journal of the Chemical Society - Chemical Communications, 1988, page 1145).

The manganese co-ordination complexes usable as new bleach catalysts of the invention may be prepared and synthesized in manners as described in literature for several manganese complexes illustrated below:

#### SYNTHESIS OF

$[Mn^{III}2(\mu-O)_1(\mu-OAc)_2(Me-TACN)_2](ClO_4)_2 \cdot (H_2O)$

(A Catalyst Precursor)

All solvents were degassed (first a vacuum was applied over the solvent for 5 minutes and subsequently argon gas was introduced; this was repeated three times) prior to use (to exclude all oxygen, which oxidizes  $Mn^{II}$  to  $Mn^{IV}$  and causes the formation of  $Mn^{IV}O_2$ ).

The reaction was carried out at room temperature, under argon atmosphere, unless otherwise stated.

In a 25 ml round-bottomed flask, equipped with a magnetic stirrer, 500 mg (2.91 mmol) 1,4,7-trimethyl-1,4,7-triazacyclononane was dissolved in 15 ml

ethanol/water (85/15). This gave a clear, colourless solution ( $pH > 11$ ). Then 0.45 g (1.80 mmol)  $Mn^{III}OAc_3 \cdot 2aq$  was added and a cloudy, dark-brown solution

was obtained. After the addition of 1.00 g (7.29 mmol)  $NaOAc \cdot 3aq$ , the pH fell to 8 and with about 15 drops of 70%  $HClO_4$  solution, the pH of the reaction mixture was adjusted to 5.0. After the addition of 1.50 g (12.24 mmol)  $NaClO_4$ , the colour of the reaction mixture changed from brown to red within about 30 minutes. After allowing the reaction mixture to stand for one week at room temperature, the product precipitated in the form of red crystals. Then the precipitate was filtered over a glass filter, washed with ethanol/water (85/15) and dried in a dessicator over KOH.

#### SYNTHESIS OF

$[Mn^{III}Mn^{IV}(\mu-O)_1(\mu-OAc)_2(Me-TACN)_2](ClO_4)_3$

(A Catalyst Precursor)

All solvents were degassed as described above, prior to use (to exclude all oxygen, which oxidizes  $Mn^{II}$  to  $Mn^{IV}$  and causes the formation of  $Mn^{IV}O_2$ ). The reaction was carried out at room temperature, under argon atmosphere, unless otherwise stated.

In a 50 ml round-bottomed flask, equipped with a magnetic stirrer, 500 mg (2.90 mmol) 1,4,7-trimethyl-1,4,7-triazacyclononane was dissolved in 9 ml ethanol. This gave a clear, colourless solution ( $pH > 11$ ). Then 0.75 g (3.23 mmol)  $Mn^{III}OAc_3 \cdot 2aq$  was added and a cloudy dark-brown solution was obtained. After the addition of 0.50 g (6.00 mmol)  $NaOAc \cdot 3aq$  and 10 ml water, the pH fell to 8. Then 1.0 ml 70%  $HClO_4$  was added ( $pH 1$ ), which started the precipitation of a brown powder that formed the product. The reaction mixture was allowed to stand for several hours at room temperature. Then the precipitate was filtered over a glass filter, washed with ethanol/water (60/40) and dried in a dessicator over KOH. In the filtrate no further precipitation was observed. The colour of the filtrate changed from green-brown to colourless in two

weeks' time. Mn(III,IV)MeTACN is a green-brown microcrystalline product.

SYNTHESIS OF  $[\text{Mn}^{IV}(\mu\text{-O})_3(\text{Me-TACN})_2](\text{PF}_6)_2 \text{H}_2\text{O}$

In a 50 ml round-bottomed flask, equipped with a magnetic stirrer, 661.4 mg of (4), i.e.  $[\text{Mn}^{III}(\mu\text{-O})_2(\mu\text{-OAc})_2(\text{Me-TACN})_2](\text{ClO}_4)_2$  (0.823 mmol crystals were pulverized, giving a purple powder) was dissolved in 40 ml of an ethanol/water mixture (1/1). After a five-minute ultrasonic treatment and stirring at room temperature for 15 minutes, all powder was dissolved, giving a dark-red-coloured neutral solution. 4 ml of triethylamine was added and the reaction mixture turned to dark-brown colour (pH > 11). Immediately 15 3.55 g of sodium hexafluorophosphate (21.12 mmol, NaPF<sub>6</sub>) was added. After stirring for 15 minutes at room temperature, in the presence of air, the mixture was filtered to remove some manganese dioxide, and the filtrate was allowed to stand overnight. A mixture of MnO<sub>2</sub> and red crystals was formed. The solids were collected by filtration and washed with ethanol. The red crystals (needles) were isolated by adding a few ml of acetonitrile to the filter. The crystals easily dissolved, while MnO<sub>2</sub>, insoluble in acetonitrile, remained on the filter. Evaporation of the acetonitrile solution resulted in the product as red flocks.

An advantage of the bleach catalysts of the invention is that they are hydrolytically and oxidatively stable, and that the complexes themselves are catalytically active, and function in a variety of detergent formulations.

Another advantage is that the instant catalysts are surprisingly much better than any other manganese complexes hitherto proposed in the art. They are furthermore not only effective in enhancing the bleaching action of hydrogen peroxide but also of organic and inorganic peroxyacid compounds.

A surprising feature of the bleach systems according to the invention is that they are effective on a wide range of stains including both hydrophilic and hydrophobic stains. This is in contrast with all previously proposed Mn-based catalysts, which are only effective on hydrophilic stains.

A further surprising feature is that they are compatible with detergent enzymes, such as proteases, cellulases, lipases, amylases, oxidases etc.

Accordingly, in one aspect, the invention provides a bleaching or cleaning process employing a bleaching agent selected from the group of peroxy compound bleaches including hydrogen peroxide, hydrogen peroxide-liberating or -generating compounds, peroxyacids and their salts, and peroxyacid bleach precursors and mixtures thereof, which process is characterized in that said bleaching agent is activated by a catalytic amount of a Mn-complex as defined hereinbefore.

The catalytic component is a novel feature of the invention. The effective level of the Mn-complex catalyst, expressed in terms of parts per million (ppm) of manganese in the aqueous bleaching solution, will normally range from 0.001 ppm to 100 ppm, preferably from 0.01 ppm to 10 ppm, most preferably from 0.05 ppm to 5 ppm. Higher levels may be desired and applied in industrial bleaching processes, such as textile and paper pulp-bleaching. The lower range levels are primarily destined and preferably used in domestic laundry operations.

In another aspect, the invention provides an improved bleaching composition comprising a peroxy compound bleach as defined above and a catalyst for the bleaching action of the peroxy compound bleach, said catalyst comprising the aforesaid Mn-complex.

As indicated above, the improved bleaching composition has particular application in detergent formulations to form a new and improved detergent bleach composition within the purview of the invention, comprising said peroxy compound bleach, the aforesaid Mn-complex catalyst, a surface-active material, and usually also detergency builders and other known ingredients of such formulations, as well as in the industrial bleaching of yarns, textiles, paper, woodpulp and the like.

The Mn-complex catalyst or precursor thereof will be present in the detergent formulations in amounts so as to provide the required level in the wash liquor. When the dosage of the detergent bleach composition is relatively low, e.g. about 1 and 2 g/1 by consumers in Japan and the USA, respectively, the Mn content in the formulation is 0.001 to 1.0%, preferably 0.005 to 0.50%. At higher product dosage as used e.g. by European consumers, the Mn content in the formulation is 0.0005 to 0.25%, preferably from 0.001 to 0.1%.

Compositions comprising a peroxy compound bleach and the aforesaid bleach catalyst are effective over a wide pH range of between 7 and 13, with optimal pH range lying between 8 and 11.

The peroxy compound bleaches which can be utilized in the present invention include hydrogen peroxide, hydrogen peroxide-liberating compounds, hydrogen peroxide-generating systems, peroxyacids and their salts, and peroxyacid bleach precursors and mixtures thereof. It is of note, however, that the invention is of particular interest in the bleach activation of hydrogen peroxide and hydrogen peroxide adducts, in which the effect is most outstanding.

Hydrogen peroxide sources are well known in the art. They include the alkali metal peroxides, organic peroxide bleaching compounds such as urea peroxide, and inorganic persalt bleaching compounds, such as the alkali metal perborates, percarbonates, perphosphates and persulphates. Mixtures of two or more such compounds may also be suitable. Particularly preferred are sodium percarbonate and sodium perborate and, especially, sodium perborate monohydrate. Sodium perborate monohydrate is preferred to tetrahydrate because of its excellent storage stability while also dissolving very quickly in aqueous bleaching solutions. Sodium percarbonate may be preferred for environmental reasons. These bleaching compounds may be utilized alone or in conjunction with a peroxyacid bleach precursor.

Peroxyacid bleach precursors are known and amply described in literature, such as in the GB Patents 836,988; 864,798; 907,356; 1,003,310 and 1,519,351; German Patent 3,337,921; EP-A-0185522; EP-A-0174132; EP-A-0120591; and U.S. Pat. Nos. 1,246,339; 3,332,882; 4,128,494; 4,412,934 and 4,675,393.

Another useful class of peroxyacid bleach precursors is that of the quaternary ammonium substituted peroxyacid precursors as disclosed in U.S. Pat. Nos. 4,751,015 and 4,397,757, in EP-A-284292, EP-A-331,229 and EP-A-0303520. Examples of peroxyacid bleach precursors of this class are:

2-(N,N,N-trimethyl ammonium) ethyl-4-sulphophenyl carbonate - (SPCC);

N-octyl,N,N-dimethyl-N<sub>10</sub>-carbophenoxy decyl ammonium chloride - (ODC);  
 3-N,N,N-trimethyl ammonium propyl sodium-4-sulphophenyl carboxylate; and  
 N,N,N-trimethyl ammonium toluyloxy benzene sulphonate.

Of the above classes of bleach precursors, the preferred classes are the esters, including acyl phenol sulphonates and acyl alkyl phenol sulphonates; acylamides; and the quaternary ammonium substituted peroxyacid precursors.

Highly preferred activators include sodium-4-benzyloxy benzene sulphonate; N,N,N',N'-tetraacetyl ethylene diamine; sodium-1-methyl-2-benzyloxy benzene-4-sulphonate; sodium-4-methyl-3-benzyloxy benzoate; SPCC trimethyl ammonium toluyloxy benzene sulphonate; sodium nonanoxyloxybenzene sulphonate; sodium 3,5,5-trimethyl hexanoxyloxybenzene sulphonate; glucose pentaacetate and tetraacetyl xylose.

Organic peroxyacids are also suitable as the peroxy compound. Such materials normally have a general formula:



wherein R is an alkylene or substituted alkylene group containing from 1 to about 22 carbon atoms or a phenylene or substituted phenylene group, and Y is hydrogen, halogen, alkyl, aryl or



The organic peroxy acids usable in the present invention can contain either or two peroxy groups and can be either aliphatic or aromatic. When the organic peroxy acid is aliphatic, the unsubstituted acid has the general formula:



where Y can be, for example, H, CH<sub>3</sub>, CH<sub>2</sub>Cl, COOH, or COOOH; and n is an integer from 1 to 20.

When the organic peroxy acid is aromatic, the unsubstituted acid has the general formula:



wherein Y is hydrogen, alkyl, alkylhalogen, halogen, or COOH or COOOH.

Typical monoperoxy acids useful herein include alkyl peroxy acids and aryl peroxy acids such as:

- (i) peroxybenzoic acid and ring-substituted peroxybenzoic acids, e.g. peroxy- $\alpha$ -naphthoic acid;
- (ii) aliphatic, substituted aliphatic and arylalkyl monoperoxy acids, e.g. peroxylauric acid, peroxystearic acid, and N,N-phthaloylaminoperoxycaproic acid.

Typical diperoxy acids useful herein include alkyl diperoxy acids and aryl diperoxy acids, such as:

- (iii) 1,12-diperoxydodecanedioic acid;
- (iv) 1,9-diperoxyazelaic acid;

(v) diperoxybrassylic acid; diperoxysebacic acid and diperoxyisophthalic acid;

(vi) 2-decyldiperoxybutane-1,4-dioic acid;

(vii) 4,4'-sulfonylbisperoxybenzoic acid.

An inorganic peroxyacid salt usable herein is, for example, potassium monopersulphate.

A detergent bleach composition of the invention can be formulated by combining effective amounts of the components. The term "effective amounts" as used herein means that the ingredients are present in quantities such that each of them is operative for its intended purpose when the resulting mixture is combined with water to form an aqueous medium which can be used to wash and clean clothes, fabrics and other articles.

In particular, the detergent bleach composition can be formulated to contain, for example, from about 2% to 30% by weight, preferably from 5 to 25% by weight, of hydrogen peroxide or a hydrogen peroxide-liberating compound.

Peroxyacids may be utilized in somewhat lower amounts, for example from 1% to about 15% by weight, preferably from 2% to 10% by weight.

Peroxyacid precursors may be utilized in combination with a peroxide compound in approximately the same level as peroxyacids, i.e. 1% to 15%, preferably from 2% to 10% by weight.

The manganese complex catalyst will be present in such formulations in amounts so as to provide the required level of Mn in the wash liquor. Normally, an amount of manganese complex catalyst is incorporated in the formulation which corresponds to a Mn content of from 0.0005% to about 1.0% by weight, preferably 0.001% to 0.5% by weight.

The bleach catalyst of the invention is compatible with substantially any known and common surface-active agents and detergency builder materials.

The surface-active material may be naturally derived, such as soap, or a synthetic material selected from anionic, nonionic, amphoteric, zwitterionic, cationic actives and mixtures thereof. Many suitable actives are commercially available and are amply described in literature, for example in "Surface Active Agents and Detergents", Volumes I and II, by Schwartz, Perry and Berch. The total level of the surface-active material may range up to 50% by weight, preferably being from about 1% to 40% by weight of the composition, most preferably 4 to 25%.

Synthetic anionic surface-actives are usually water-soluble alkali metal salts of organic sulphates and sulphonates having alkyl groups containing from about 8 to about 22 carbon atoms, the term alkyl being used to include the alkyl portion of higher aryl groups.

Examples of suitable synthetic anionic detergent compounds are sodium and ammonium alkyl sulphates, especially those obtained by sulphating higher (C<sub>8</sub>-C<sub>18</sub>) alcohols produced, for example, from tallow or coconut oil; sodium and ammonium alkyl (C<sub>9</sub>-C<sub>20</sub>) benzene sulphonates, particularly sodium linear secondary alkyl (C<sub>10</sub>-C<sub>15</sub>) benzene sulphonates; sodium alkyl glyceryl ether sulphates, especially those esters of the higher alcohols derived from tallow or coconut oil and synthetic alcohols derived from petroleum; sodium coconut oil fatty acid monoglyceride sulphates and sulphonates; sodium and ammonium salts of sulphuric acid esters of higher (C<sub>9</sub>-C<sub>18</sub>) fatty alcohol alkylene oxide, particularly ethylene oxide, reaction products; the reaction products of fatty acids such as coconut fatty acids esterified with isethionic acid and neutralized with so-

dium hydroxide; sodium and ammonium salts of fatty acid amides of methyl taurine; alkane monosulphonates such as those derived by reacting alpha-olefins (C<sub>8</sub>-C<sub>20</sub>) with sodium bisulphite and those derived by reacting paraffins with SO<sub>2</sub> and Cl<sub>2</sub> and then hydrolyzing with a base to produce a random sulphonate; sodium and ammonium C<sub>7</sub>-C<sub>12</sub> dialkyl sulfosuccinates; and olefin sulphonates, which term is used to describe the material made by reacting olefins, particularly C<sub>10</sub>-C<sub>20</sub> alpha-olefins, with SO<sub>3</sub> and then neutralizing and hydrolyzing the reaction product. The preferred anionic detergent compounds are sodium (C<sub>11</sub>-C<sub>15</sub>) alkylbenzene sulphonates, sodium (C<sub>16</sub>-C<sub>18</sub>) alkyl sulphates and sodium (C<sub>16</sub>-C<sub>18</sub>) alkyl ether sulphates.

Examples of suitable nonionic surface-active compounds which may be used, include in particular the reaction products of alkylene oxides, usually ethylene oxide, with alkyl (C<sub>6</sub>-C<sub>22</sub>) phenols, generally 5-25 EO, i.e. 5-25 units of ethylene oxides per molecule; the condensation products of aliphatic (C<sub>8</sub>-C<sub>18</sub>) primary or secondary linear or branched alcohols with ethylene oxide, generally 3-30 EO, and products made by condensation of ethylene oxide with the reaction products of propylene oxide and ethylene diamine. Other so-called nonionic surface-actives include alkyl polyglycosides, long chain tertiary amine oxides, long chain tertiary phosphine oxides and dialkyl sulphoxides.

Amounts of amphoteric or zwitterionic surface-active compounds can also be used in the compositions of the invention but this is not normally desired owing to their relatively high cost. If any amphoteric or zwitterionic detergent compounds are used, it is generally in small amounts in compositions based on the much more commonly used synthetic anionic and nonionic actives.

As stated above, soaps may also be incorporated in the compositions of the invention, preferably at a level of less than 25% by weight. They are particularly useful at low levels in binary (soap/anionic) or ternary mixtures together with nonionic or mixed synthetic anionic and nonionic compounds. Soaps which are used, are preferably the sodium, or, less desirably, potassium salts of saturated or unsaturated C<sub>10</sub>-C<sub>24</sub> fatty acids or mixtures thereof. The amount of such soaps can be varied between about 0.5% and about 25% by weight, with lower amounts of about 0.5% to about 5% being generally sufficient for lather control. Amounts of soap between about 2% and about 20%, especially between about 5% and about 10%, are used to give a beneficial effect on detergency. This is particularly valuable in compositions used in hard water when the soap acts as a supplementary builder.

The detergent compositions of the invention will normally also contain a detergency builder. Builder materials may be selected from 1) calcium sequestrant materials, 2) precipitating materials, 3) calcium ion-exchange materials and 4) mixtures thereof.

Examples of calcium sequestrant builder materials include alkali metal polyphosphates, such as sodium tripolyphosphate; nitrilotriacetic acid and its water-soluble salts; the alkali metal salts of ether polycarboxylates, such as carboxymethoxy succinic acid, oxydysuccinic acid, mellitic acid; ethylene diamine tetraacetic acid; benzene polycarboxylic acids; citric acid; and polyacetal carboxylates as disclosed in U.S. Pat. Nos. 4,144,226 and 4,146,495.

Examples of precipitating builder materials include sodium orthophosphate, sodium carbonate and sodium carbonate/calcite.

Examples of calcium ion-exchange builder materials include the various types of water-insoluble crystalline or amorphous aluminosilicates, of which zeolites are the best known representatives.

In particular, the compositions of the invention may contain any one of the organic or inorganic builder materials, such as sodium or potassium tripolyphosphate, sodium or potassium pyrophosphate, sodium or potassium orthophosphate, sodium carbonate or sodium carbonate calcite mixtures, the sodium salt of nitrilotriacetic acid, sodium citrate, carboxymethyl malonate, carboxymethoxy succinate and the water-insoluble crystalline or amorphous aluminosilicate builder materials, or mixtures thereof.

These builder materials may be present at a level of, for example, from 5 to 80% by weight, preferably from 10 to 60% by weight.

Apart from the components already mentioned, the detergent compositions of the invention can contain any of the conventional additives in the amounts in which such materials are normally employed in fabric washing detergent compositions. Examples of these additives include lather boosters, such as alkanolamides, particularly the monoethanol amides derived from palmkernel fatty acids and coconut fatty acids, lather depressants, such as alkyl phosphates and silicones, anti-redeposition agents, such as sodium carboxymethyl cellulose and alkyl or substituted alkyl cellulose ethers, other stabilizers, such as ethylene diamine tetraacetic acid and the phosphonic acid derivatives (i.e. Dequest® types), fabric softening agents, inorganic salts, such as sodium sulphate, and, usually present in very small amounts, fluorescent agents, perfumes, enzymes, such as proteases, cellulases, lipases, amylases and oxidases, germicides and colourants.

Another optional but highly desirable additive ingredient with multi-functional characteristics in detergent compositions is from 0.1% to about 5% by weight of a polymeric material having a molecular weight of from 1,000 to 2,000,000 and which can be a homo- or copolymer of acrylic acid, maleic acid, or salt or anhydride thereof, vinyl pyrrolidone, methyl- or ethyl-vinyl ethers, and other polymerizable vinyl monomers. Preferred examples of such polymeric materials are polyacrylic acid or polyacrylate; polymaleic acid/acrylic acid copolymer; 70:30 acrylic acid/hydroxyethyl maleate copolymer; 1:1 styrene/maleic acid copolymer; isobutylene/maleic acid and diisobutylene/maleic acid copolymers; methyl- and ethyl-vinylether/maleic acid copolymers; ethylene/maleic acid copolymer; polyvinyl pyrrolidone; and vinyl pyrrolidone/maleic acid copolymer.

Detergent bleach compositions of the invention formulated as free-flowing particles, e.g. in powdered or granulated form, can be produced by any of the conventional techniques employed in the manufacture of detergent compositions, for instance by slurry-making, followed by spray-drying to form a detergent base powder to which the heat-sensitive ingredients including the peroxy compound bleach and optionally some other ingredients as desired, and the bleach catalyst, can be added as dry substances.

It will be appreciated, however, that the detergent base powder compositions, to which the bleach catalyst is added, can itself be made in a variety of other ways, such as the so-called part-part processing, non-tower route processing, dry-mixing, agglomeration, granulation, extrusion, compacting and densifying processes

etc., such ways being well known to those skilled in the art and not forming the essential part of the present invention.

Alternatively, the bleach catalyst can be added separately to a wash/bleach water containing the peroxy compound bleaching agent.

In that case, the bleach catalyst is presented as a detergent additive product. Such additive products are intended to supplement or boost the performance of conventional detergent compositions and may contain any of the components of such compositions, although they will not comprise all of the components as present in a fully formulated detergent composition. Additive products in accordance with this aspect of the invention will normally be added to an aqueous liquid containing a source of (alkaline) hydrogen peroxide, although in certain circumstances the additive product may be used as separate treatment in a pre-wash or in the rinse.

Additive products in accordance with this aspect of the invention may comprise the compound alone or, preferably, in combination with a carrier, such as a compatible aqueous or non-aqueous liquid medium or a particulate substrate or a flexible non-particulate substrate.

Examples of compatible particulate substrates include inert materials, such as clays and other aluminosilicates, including zeolites, both natural and synthetic of origin. Other compatible particulate carrier materials include hydratable inorganic salts, such as carbonates and sulphates.

The instant bleach catalyst can also be formulated in detergent bleach compositions of other product forms, such as flakes, tablets, bars and liquids, particularly non-aqueous liquid detergent compositions.

Such non-aqueous liquid detergent compositions in which the instant bleach catalyst can be incorporated are known in the art and various formulations have been proposed, e.g. in U.S. Pat. Nos. 2,864,770; 3,368,977; 4,772,412; GB Patents 1,205,711; 1,370,377; 2,194,536; DE-A-2,233,771 and EP-A-0,028,849.

These are compositions which normally comprise a non-aqueous liquid medium, with or without a solid phase dispersed therein. The non-aqueous liquid medium may be a liquid surfactant, preferably a liquid nonionic surfactant; a polar solvent, e.g. polyols, such as glycerol, sorbitol, ethylene glycol, optionally combined with low-molecular monohydric alcohols, e.g. ethanol or isopropanol; or mixtures thereof.

The solid phase can be builders, alkalis, abrasives, polymers, clays, other solid ionic surfactants, bleaches, fluorescent agents and other usual solid detergent ingredients.

The invention will now be further illustrated by way of the following non-limiting Examples.

## EXAMPLES

The experiments were either carried out in a temperature-controlled glass beaker equipped with a magnetic stirrer, thermocouple and a pH electrode, or under real washing machine conditions.

### GLASS-VESSEL EXPERIMENTAL CONDITIONS

Most of the experiments were carried out at a constant temperature of 40° C.

In the experiments, demineralised water, hardened-up demineralised or tap water (16°FH) was applied. A Ca/Mg stock solution Ca:Mg=4:1 (weight ratio) was used to adjust water hardness.

In Examples, when formulations were used, the dosage amounted to about 6 g/l total formulation. The compositions of the base detergent formulations without bleach used are described below.

The amount of sodium perborate monohydrate was about 15%, yielding 8.6 mmol/l H<sub>2</sub>O<sub>2</sub>, calculated on 6 g/l dosage.

In most cases the catalysts were dosed at a concentration of between 10<sup>-6</sup> to 10<sup>-5</sup> mol Mn/l.

In experiments at 40° C. the initial pH was adjusted to 10.5.

Tea-stained cotton test cloth was used as bleach monitor. After rinsing in tap water, the cloths were dried in a tumble drier. The reflectance (R<sub>460\*</sub>) was measured before and after washing on a Zeiss Elrephometer. The average was taken of 2 values/test cloth.

### DETERGENT FORMULATIONS WITHOUT BLEACH (%)

|                                         | A  | B  | C  | D  | E  |
|-----------------------------------------|----|----|----|----|----|
| Anionic surfactant                      | 13 | 12 | 13 | 8  | 7  |
| Nonionic surfactant                     | 5  | 13 | 5  | 13 | 8  |
| Sodium triphosphate                     | 40 | —  | —  | —  | —  |
| Zeolite                                 | —  | 39 | —  | 35 | 27 |
| Polymer                                 | —  | 6  | —  | 5  | 3  |
| Sodium carbonate                        | —  | 15 | 36 | 16 | 11 |
| Calcite                                 | —  | —  | 24 | —  | —  |
| Sodium silicate                         | 8  | —  | 7  | 1  | 1  |
| Na <sub>2</sub> SO <sub>4</sub>         | 20 | —  | —  | —  | 27 |
| Savinase ® granule (proteolytic enzyme) | —  | —  | —  | 1  | 1  |
| Water and minors                        | 14 | 15 | 15 | 22 | 15 |

### EXAMPLE I

The bleach performance of some manganese catalysts of the invention is compared with that of other Co- and Mn-based catalysts.

Conditions: Glass-vessel experiments; no detergent formulation; demineralised water; T=40° C.; t=60 minutes; pH=10.5; [H<sub>2</sub>O<sub>2</sub>]=8.6×10<sup>-3</sup> mol/l.

| Catalyst                                                                                                              | Metal concentration<br>mol/l | ΔR <sub>460*</sub> (15 min) | ΔR <sub>460*</sub> (60 min) |
|-----------------------------------------------------------------------------------------------------------------------|------------------------------|-----------------------------|-----------------------------|
| CoCo*                                                                                                                 | —                            | 1                           | 7                           |
| Mn <sup>II</sup> (CF <sub>3</sub> SO <sub>3</sub> ) <sub>2</sub>                                                      | 12×10 <sup>-6</sup>          | 9                           | 22                          |
| Mn <sup>III</sup> gluconate                                                                                           | 6×10 <sup>-6</sup>           | 4                           | 16                          |
| Mn <sup>III</sup> (μ-O)(μ-OAc) <sub>2</sub> (Me-TACN) <sub>2</sub> -(ClO <sub>4</sub> ) <sub>2</sub>                  | 5×10 <sup>-6</sup>           | 4                           | 16                          |
| Mn <sup>III</sup> Mn <sup>IV</sup> (μ-O)(μ-OAc) <sub>2</sub> (Me-TACN) <sub>2</sub> -(ClO <sub>4</sub> ) <sub>3</sub> | 2.5×10 <sup>-6</sup>         | 14                          | 29                          |
| Mn <sup>IV</sup> (μ-O) <sub>3</sub> (Me-TACN) <sub>2</sub> -(PF <sub>6</sub> ) <sub>2</sub>                           | 3.4×10 <sup>-6</sup>         | 16                          | 31                          |
| Mn <sup>IV</sup> <sub>2</sub> (μ-O) <sub>3</sub> (Me/Me-TACN) <sub>2</sub> -(PF <sub>6</sub> ) <sub>2</sub>           | 3.7×10 <sup>-6</sup>         | 19                          | 33                          |
|                                                                                                                       | 6×10 <sup>-6</sup>           | 17                          | 30                          |

\*CoCo is an abbreviation for 11,23-dimethyl-3,7,15,19-tetraazatricyclo [19.3.1.1.9,13] hexacosa - 2,7,9,11,13 (26), 14,19,21 (25), 22,24-decane-25,26-diolate-Co<sub>2</sub>Cl<sub>2</sub> (described in EP-A-0408131).

The results clearly demonstrate the superior performance of the new Mn-catalysts over the system without catalysts and other Mn- and Co-based catalysts.

#### EXAMPLE II

In this Example the bleach performance of a manganese catalyst of the invention is compared with that of other manganese catalysts at the same concentration.

Conditions: Glass-vessel experiments; no detergent formulation; Demin. water,  $t=30$  min.,  $T=40^\circ C$ ,  $pH=10.5$  and  $[H_2O_2]=8.6 \times 10^{-3} \text{ mol/l}$ .

| Catalyst                                  | Mn-concentration<br>mol/l | $\Delta R_{460}$ |
|-------------------------------------------|---------------------------|------------------|
| $Mn^{II}Cl_2$                             | $1.10^{-5}$               | 4                |
| $Mn^{III}$ gluconate                      | $1.10^{-5}$               | 9                |
| $Mn$ -sorbitol <sub>3</sub>               | $1.10^{-5}$               | 10               |
| $[Mn^{IV}_2(\mu-O)_3(Me-TACN)_2](PF_6)_2$ | $1.10^{-5}$               | 29               |

These results show the clearly superior bleach catalysis of the  $[Mn^{IV}_2(\mu-O)_3(Me-TACN)_2](PF_6)_2$  catalyst over the previously known Mn-based catalyst at the same manganese concentration.

#### EXAMPLE III

This Example shows the effect of  $[Mn^{III}_2(\mu-O)_1(\mu-OAc)_2(Me-TACN)_2](ClO_4)_2$  catalyst precursor concentration on the bleach performance.

Conditions: Glass-vessel experiments; no detergent formulation;  $T=40^\circ C$ ,  $t=30$  minutes,  $pH=10.5$ , demin. water, and  $[H_2O_2]=8.6 \times 10^{-3} \text{ mol/l}$ .

| Mn-concentration in mol/l | $\Delta R_{460}^*$ |
|---------------------------|--------------------|
| $10^{-7}$                 | 4                  |
| $10^{-6}$                 | 8                  |
| $2 \times 10^{-6}$        | 17                 |
| $5 \times 10^{-6}$        | 21                 |
| $10^{-5}$                 | 26                 |
|                           | 29                 |

The results show the strong catalytic effect already at a very low concentration and over a broad concentration range.

#### EXAMPLE IV

The bleach performance of different catalysts at  $20^\circ C$  are compared.

Conditions: Glass-vessel experiments; no detergent formulation; Demin. water,  $T=20^\circ C$ ,  $t=60$  minutes;  $pH 10.5$ ;  $[H_2O_2]=8.6 \times 10^{-3} \text{ mol/l}$ ,  $[metal]=10^{-5} \text{ mol/l}$ .

| Catalyst                                  | $\Delta R_{460}^*$ |
|-------------------------------------------|--------------------|
| $Mn$ -sorbitol <sub>3</sub>               | 2                  |
| $CoCo^*$                                  | 3                  |
| $Co^{III}(NH_3)_5Cl^{**}$                 | 7                  |
| $[Mn^{IV}_2(\mu-O)_3(Me-TACN)_2](PF_6)_2$ | 8                  |
|                                           | 20                 |

$CoCo^*$  - for description see Example I.

$Co^{III}(NH_3)_5Cl^{**}$  - Cobalt catalyst described in EP-A-0272030 (Interox).

The above results show that the present catalyst still performs quite well at  $20^\circ C$ , at which temperature

other known catalysts do not seem to be particularly effective.

#### EXAMPLE V

The bleach of the  $Mn^{III}_2(\mu-O)_1(\mu-OAc)_2(Me-TACN)_2$  catalyst precursor is shown as a function of temperature.

Conditions: Glass-vessel experiments; no detergent formulation; Demin. water,  $pH=10$ ,  $t=20$  minutes,  $[Mn]=10^{-5} \text{ mol/l}$ ,  $[H_2O_2]=8.6 \times 10^{-3} \text{ mol/l}$ .

| Temperature $^\circ C$ . | Catalyst |    |
|--------------------------|----------|----|
|                          | -        | +  |
| 20                       | 1        | 9  |
| 30                       | 2        | 15 |
| 40                       | 3        | 23 |
| 50                       | 5        | 28 |
| 60                       | 7        | 30 |

The results show that the catalyst is effective over a broad temperature range.

#### EXAMPLE VI

This Example shows the bleach catalysis of  $Mn^{III}_2(\mu-O)_1(\mu-OAc)_2(Me-TACN)_2$  catalyst precursor in different powder formulations.

Conditions: Glass-vessel experiments;  $T=40^\circ C$ ;  $t=30$  minutes;  $pH=10.5$ ; demin. water; dosage 6 g/l of detergent formulation incl. 14.3% perborate monohydrate;  $[Mn]=2.3 \times 10^{-6} \text{ mol/l}$ .

| Product<br>Formulation | Catalyst |    |
|------------------------|----------|----|
|                        | -        | +  |
| —                      | 4        | 21 |
| (A)                    | 4        | 13 |
| (B)                    | 4        | 22 |
| (C)                    | 3        | 18 |

From the above it is clear that the bleach catalysis can be obtained in very different types of formulations, e.g. with zeolite, carbonate and sodium tripolyphosphate as builders.

#### EXAMPLE VII

The effect of  $[Mn^{IV}_2(\mu-O)_3(Me-TACN)_2]$  catalyst on the stability of various detergent enzymes during the wash was examined.

Conditions: Glass-vessel experiments;  $40^\circ C$ ; 65 min.; 16°FH tap water; 5 g/l total dosage (detergent formulation D without or with 17.2% Na-perborate monohydrate (yielding  $8.6 \times 10^{-3} \text{ mol/l}$   $H_2O_2$ ); — or + catalyst at concentration  $2.5 \times 10^{-6} \text{ mol/l}$ ; — or + enzyme, activity proteases  $\sim 95 \text{ GU/ml}^*$ , lipase  $\sim 3 \text{ LU/ml}^{**}$ .

The change of enzyme activity during the experiments is expressed as time-integrated activity fraction (t.i.a.f.), i.e. the ratio of the surfaces under the curve enzyme activity vs time (i.e. 65 min.) and under the theoretical curve enzyme activity vs time (i.e. 65 min.) if no enzyme deactivation would occur.

|             | Bleaching performance<br>ΔR 460* |           |                  | Enzyme stability<br>t.i.a.f. |           |                  |
|-------------|----------------------------------|-----------|------------------|------------------------------|-----------|------------------|
|             | No bleach                        | Perborate | Perborate + cat. | No bleach                    | Perborate | Perborate + cat. |
| Savinase*** | 0                                | 6         | 24               | 0.80                         | 0.69      | 0.72             |
| Durazym***  | 0                                | 7         | 25               | 0.88                         | 0.85      | 0.77             |
| Esperase*** | 0                                | 7         | 23               | 0.92                         | 0.79      | 0.74             |
| Primase***  | 0                                | 6         | 22               | 0.91                         | 0.83      | 0.77             |
| Lipolase*** | 0                                | 7         | 26               | 0.99                         | 0.63      | 0.66             |

These figures show that the strong bleaching system of perborate + catalyst has no deleterious effect on the enzyme stability during the wash.

\*This specification of glycine units (GU) is defined in EP 0 405 901 (Unilever).

\*\*This specification of lipase units (LU) is defined in EP 0 258 068 (NOVO).

\*\*\*Commercially available enzymes from NOVO NORDISK.

### EXAMPLE VIII

The effect of  $[\text{Mn}^{IV}_2(\mu\text{-O})_3(\text{Me-TACN})_2]$  on the bleaching performance of peracids and precursor/perborate systems. The precursors used in the experiments are N,N,N',N'-tetraacetyl ethylene diamine (TAED) 20 and SPCC.

#### VIII A

Conditions: Glass-vessel experiments; no detergent formulation present; 40° C.; 30 min.; pH 10.5; demin. water;  $[\text{cat}] = 2.5 \times 10^{-6}$  mol/l;  $[\text{peracid}] = 8 \times 10^{31}$  25 mol/l.

|                        | Catalyst |    | ΔR460* |
|------------------------|----------|----|--------|
|                        | -        | +  |        |
| Peracetic acid         | 9        | 20 |        |
| Sodium monopersulphate | 13       | 22 |        |

From these data it is clear that bleach catalysis is obtained with organic and inorganic peracid compounds.

#### VIII B

Conditions: Glass-vessel experiments; 40° C.; 30 min.; pH 10.0; 16°FH tap water; 6 g/l total dosage (detergent formulation D with 7.5/2.3/0.07% Na-perborate monohydrate/TAED/Dequest® 2041; - or +  $[\text{Mn}^{IV}_2(\mu\text{-O})_3(\text{Me-TACN})_2]$ ,  $[\text{cat}] = 2.5 \times 10^{-6}$  mol/l.

| Catalyst | - | +  |
|----------|---|----|
| AR 460*  | 6 | 20 |

This Example shows that the performance of a TAED/perborate bleaching system is also significantly improved by employing the catalyst.

#### VIII C

Conditions: Glass-vessel experiments; 20° C.; 30 min.; pH 10; 16°FH tap water; 6 g/l total dosage (detergent formulation D with 7.5/6.1% Na-perborate monohydrate/SPCC; - or +  $[\text{Mn}^{IV}_2(\mu\text{-O})_3(\text{Me-TACN})_2]$ ,  $[\text{cat}] = 2.5 \times 10^{-6}$  mol/l.

| Catalyst | -  | +  |
|----------|----|----|
| R 460*   | 14 | 17 |

From these data it is clear that, even at 20° C., with a precursor (SPCC)/perborate bleaching system, a signif-

icant improvement of the bleach performance can be obtained.

### EXAMPLE IX

This Example shows the bleach performance on different stains, i.e. under practical machine washing conditions as compared with the current commercial bleach system containing TAED (tetraacetyl ethylene diamine).

Conditions: Miele W 736 washing machine; 40° C. (nominal) extended wash (120 min.) cycle, 56 min. at 36° C. max; 16°FH tap water; 3 kg medium-soiled cotton load including the bleach monitors; 100 g/run total dosage (detergent formulation E, either with 14.3% Na-perborate monohydrate +0.04%  $(\mu\text{-O})_3(\text{Me-TACN})_2$  or the current bleach system 7.5/2.3/0.24% Na-perborate monohydrate/TAED/Dequest 2041.

"Dequest" is a Trademark for polyphosphonates ex Monsanto.

| STAIN                 | Reflectance Values (ΔR 460*) |        |
|-----------------------|------------------------------|--------|
|                       | Current                      | Mn-cat |
| EMPA 116 (blood/milk) | 18                           | 23     |
| EMPA 114 (wine)       | 29                           | 36     |
| BC-1 (tea)            | 7                            | 20     |
| AS-10 (casein)        | 31                           | 30     |

|               | Stain removal<br>(lower figure is better result) |    |
|---------------|--------------------------------------------------|----|
|               | Current                                          | Mn |
| Ketchup       | 28                                               | 19 |
| Curry         | 25                                               | 10 |
| Black currant | 39                                               | 18 |

The results show that the catalyst of the invention performs better than the current TAED system on different test cloths and stains and that protease activity is not negatively affected (vide AS10 results).

### EXAMPLE X

Hydrolytic stability of the catalysts of the invention is defined in terms of the water-solubility of the manganese at a pH of 10-11, in the presence of hydrogen peroxide, at a concentration of  $1.7 \times 10^{-2}$  mol/l. A  $10^{-3}$  molar solution of the Mn-complex is prepared, the pH is raised to 11 with 1N NaOH, and hydrogen peroxide is added. The transparency at 800 nm is monitored for the next 2 hours by a UV/VIS spectrophotometer (Shimadzu). If no significant decrease of transparency (or increase of adsorption) is observed, the complex is defined as hydrolytically stable.

## Sample

## Hydrolytic stability

Conditions: Glass-vessel experiments; no detergent formulation; Demin. water,  $t=30$  minutes,  $T=40^\circ C$ ;  $pH=10.5$  and  $[H_2O_2]=8.6 \times 10^{-3}$  mol/l.

| Catalyst                                         | Concentration mol/l | Mn        | $\Delta R_{460}$ |
|--------------------------------------------------|---------------------|-----------|------------------|
| $Mn^{IV}2(\mu-O)_3(Me-TACN)_2$                   | (1)                 | $10^{-5}$ | 30               |
| $Mn^{III}2(\mu-O)_1(\mu-OAc)_2(Me-TACN)_2$       | (3)                 | $10^{-5}$ | 29               |
| $Mn^{IV}Mn^{III}(\mu-O)_1(\mu-OAc)_2(Me-TACN)_2$ | (4)                 | $10^{-5}$ | 30               |

|                                                                  |     |
|------------------------------------------------------------------|-----|
| $Mn^{III}2(\mu-O)_1(\mu-OAc)_2(Me-TACN)_2$ (precursor) (3)       | Yes |
| $Mn^{III}Mn^{IV}(\mu-O)_1(\mu-OAc)_2(Me-TACN)_2$ (precursor) (4) | Yes |
| $Mn^{IV}2(\mu-O)_3(Me-TACN)_2$ (1)                               | Yes |
| $Mn^{IV}2(\mu-O)_3(Me/Me-TACN)_2$ (2)                            | Yes |

From these data it can be seen that the new manganese catalysts meet the requirement of hydrolytic stability and are suitable for use according to the present invention.

## EXAMPLE XI

Oxidative stability of the catalysts of the invention is defined in terms of water-solubility and homogeneity at a pH of 10 to 11, in the presence of strongly oxidizing agents such as hypochlorite. Oxidative stability tests are run with a  $5.10^{-5}$  molar solution of the Mn-complex at a pH of 10 to 11. After addition of a similar volume of  $10^{-3}$  molar hypochlorite, the transparency was measured as described hereinbefore (see Example X).

| Sample                                | Oxidative stability |
|---------------------------------------|---------------------|
| $Mn^{IV}2(\mu-O)_3(Me-TACN)_2$ (1)    | Yes                 |
| $Mn^{IV}2(\mu-O)_3(Me/Me-TACN)_2$ (2) | Yes                 |

From the above data, it can be seen that both  $Mn^{IV}$ -complexes of the invention meet the requirements of oxidative stability as can happen in the presence of hypochlorite.

## EXAMPLE XII

Dispenser stability of the catalysts of the invention is defined as stability against coloured manganese (hydroxide) formation in a wetted powder detergent formulation.

An amount of 3 mg of the catalyst is carefully mixed with 0.2 g of a product composed of 18 g detergent formulation B, 2.48 g Na-sulphate and 3.52 g Na-perborate monohydrate. Finally, 0.2 ml water is added to the mixture. After 10 minutes, the remaining slurry is observed upon discolourization.

| Sample                                | Stability |
|---------------------------------------|-----------|
| $Mn^{IV}2(\mu-O)_3(Me-TACN)_2$ (1)    | Yes       |
| $Mn^{IV}2(\mu-O)_3(Me/Me-TACN)_2$ (2) | Yes       |

## EXAMPLE XIII

This Example demonstrates again that it is possible to use a dinuclear anti-ferromagnetically coupled  $Mn^{IV}$  catalyst as described in the patent, or a precursor thereof, i.e. a manganese complex that is transformed into the described catalysts during the first period of the wash process.

## EXAMPLE XIV

The bleach performance of some manganese dinuclears lying outside the scope of the invention, containing a tetra-N-dentate or bi-N-dentate ligands, is compared with the performance of a tri-N-dentate containing manganese (IV) dinuclear compound of the invention.

Conditions: Glass-vessel experiments; no detergent formulation; Demin. water,  $t=30$  minutes,  $T=40^\circ C$ ;  $pH=10.5$  and  $[H_2O_2]=8.6 \times 10^{-3}$  mol/l.

| Catalyst                                                               | Mn-concentration mol/l | $\Delta R_{460}$ |
|------------------------------------------------------------------------|------------------------|------------------|
| $[N_4Mn^{III}(\mu-O)_2Mn^{IV}N_4]^+(\text{ClO}_4)_-$                   | $10^{-5}$              | 17               |
| $[\text{Bipy}_2Mn^{III}(\mu-O)_2Mn^{IV}\text{bipy}_2](\text{ClO}_4)_3$ | $10^{-5}$              | 16               |
| $[\text{Mn}_2^{IV}(\mu-O)_3(\text{Me-TACN})_2](\text{PF}_6)_2$         | $10^{-5}$              | 30               |



These results demonstrate the superior performance of the class of catalysts described, i.e. dinuclear  $Mn^{IV}$  complexes (anti-ferromagnetically coupled) with N<sub>3</sub> ligands over dinuclear manganese complexes containing ligands co-ordinating via 2×2 or 4 N-atoms, which are not the  $Mn^{IV}$  complexes (nor precursors thereof) according to the invention.

## EXAMPLE XV

Conditions: Glass-vessel experiments; no detergent formulation; Demin. water,  $t=60$  minutes,  $T=40^\circ C$ ;  $pH=10.5$ ,  $[H_2O_2]=8.6 \times 10^{-3}$  mol/l.

The bleach performance of a tetra-nuclear, ferromagnetically coupled  $Mn^{IV}$  catalyst is compared with that of a dinuclear anti-ferromagnetically coupled manganese (IV) catalyst as described in this patent.

| Catalyst                                     | Metal concentration  | $\Delta R_{460}$ |
|----------------------------------------------|----------------------|------------------|
| $[Mn^{IV}4(\mu-O)_6(\text{TACN})_4]^{4+}$    | $10 \times 10^{-6}$  | 19               |
| $[Mn^{IV}2(\mu-O)_3(\text{Me-TACN})_2]^{2+}$ | $6.4 \times 10^{-6}$ | 29               |

These results demonstrate the superior performance of the dinuclear anti-ferromagnetically coupled  $Mn^{IV}$  clusters over the tetranuclear ferromagnetically coupled manganese(IV) cluster.

We claim:

1. A bleaching composition comprising a peroxy compound present in an effective amount to accomplish bleaching or cleaning and a catalyst present in an effective amount to activate the peroxy compound, the catalyst being a manganese-based coordination complex with a general formula:



wherein Mn is manganese in the IV-oxidation state; n and m are independent integers from 2 to 8; X represents a coordination or bridging species; p is an integer from 0 to 32; Y is a counterion, the type of which is dependent upon the charge z of the complex; q=z/[charge Y]; and L is a ligand which is an organic molecule containing a number of hetero-atoms selected from the group consisting of N, P, O and S which coordinates via at least some of said hetero-atoms to at least one Mn<sup>IV</sup>-center, and wherein at least two manganese atoms are anti-ferromagnetically coupled.

2. A composition according to claim 1, further comprising from about 1% to 50% by weight of a surfactant.

3. A composition according to claim 1, wherein the catalyst is [Mn<sup>IV</sup><sub>2</sub>(μ-O)<sub>3</sub>(Me-TACN)<sub>2</sub>](PF<sub>6</sub>)<sub>2</sub>.

4. A composition according to claim 1, wherein the catalyst is [Mn<sup>IV</sup><sub>2</sub>(μ-O)<sub>3</sub>(Me/Me-TACN)<sub>2</sub>](PF<sub>6</sub>)<sub>2</sub>.

5. A composition according to claim 1, which comprise said peroxy compound at a level of from 2 to 30% by weight and said catalyst at a level corresponding to a manganese content of from 0.0005% to 1.0% by weight.

6. A composition according to claim 5, wherein said manganese content is from 0.001% to 0.5% by weight.

7. A composition according to claim 1, wherein said peroxy compound is selected from the group consisting of hydrogen peroxide, hydrogen peroxide-liberating compounds, hydrogen peroxide-generating systems, peroxyacids and their salts, and mixtures thereof.

8. A composition according to claim 7, wherein the peroxyacid is N,N-phthaloylaminoperoxyacrylic acid.

9. A composition according to claim 7, which further comprises an enzyme selected from the group consisting of proteases, cellulases, lipases, amylases, oxidases and mixtures thereof.

10. A composition according to claim 7, which further comprises a surface-active material in an amount up to 50% by weight.

11. A composition according to claim 10, which further comprises a detergency builder in an amount of from 5 to 80% by weight.

12. A method for bleaching or cleaning of a substrate comprising contacting the substrate with a peroxy compound present in an effective amount to accomplish the bleaching or cleaning and a catalyst present in an effective amount to activate the peroxy compound, the catalyst being a manganese-based coordination complex with a general formula:



wherein Mn is manganese in the IV-oxidation state; n and m are independent integers from 2 to 8; X represents a coordination or bridging species; p is an integer from 0 to 32; Y is a counterion, the type of which is dependent upon the charge z of the complex; q=z/[charge Y]; and L is a ligand which is an organic molecule containing a number of hetero-atoms selected from the group consisting of N, P, O and S which coordinates via at least some of said hetero-atoms to at least one Mn<sup>IV</sup>-center, and wherein at least two manganese atoms are anti-ferromagnetically coupled.

20 13. A method according to claim 12 wherein the substrate is selected from the group consisting of laundry, dishes, textiles, paper and wood pulp.

25 14. A method according to claim 12, wherein said catalyst is used at a level of from 0.001 ppm to 100 ppm of manganese in a bleaching solution.

30 15. A method according to claim 14, wherein said level of manganese is from 0.01 to 20 ppm.

35 16. A method according to claim 12, wherein said bleaching agent is selected from the group consisting of hydrogen peroxide, hydrogen peroxide-liberating compounds, hydrogen peroxide-generating systems, peroxyacids and their salts, and mixtures thereof.

40 17. A method according to claim 16, wherein the peroxyacid is N,N-phthaloylaminoperoxyacrylic acid.

18. A method according to claim 16, wherein the catalyst is [Mn<sup>IV</sup><sub>2</sub>(μ-O)<sub>3</sub>(Me-TACN)<sub>2</sub>](PF<sub>6</sub>)<sub>2</sub>.

45 19. A method according to claim 16, wherein the catalyst is [Mn<sup>IV</sup><sub>2</sub>(μ-O)<sub>3</sub>(Me/Me-TACN)<sub>2</sub>](PF<sub>6</sub>)<sub>2</sub>.

\* \* \* \* \*